

# UNITED STATES PATENT OFFICE.

WILBRAHAM EVELYN LIARDÉT, OF CAMBRIA, NEW SOUTH WALES.

## MANUFACTURE OF EXPLOSIVES.

SPECIFICATION forming part of Letters Patent No. 417,429, dated December 17, 1889.

Application filed August 13, 1889. Serial No. 320,661. (No specimens.) Patented in South Australia July 12, 1889, No. 1,356.

*To all whom it may concern:*

Be it known that I, WILBRAHAM EVELYN LIARDÉT, inventor, a subject of the Queen of Great Britain, residing at Cambria, Darling Street, Balmain, in the Colony of New South Wales, Australia, have invented an Improved Process of Manufacturing Explosive Compounds, (for which I have received Letters Patent in South Australia, dated July 12, 1889, No. 1,356,) of which the following is a full, clear, and exact description.

My invention relates to the manufacture of an explosive compound containing as ingredients picric acid combined with nitrate of potash or other similar substances producing the like effect in combination.

It consists in part in eliminating during the process of manufacture the elements of danger hitherto attending such manufacture by first reducing the picric acid in glycerine, which deprives the compound of its detonating properties and renders it harmless at all stages of its manufacture; further, the volume or quantity of glycerine in my process being eighteen times less than the quantity of water used by the ordinary method of mixing and combining picric acid, I obtain better results as regards both quantity and quality.

By means of my process I shorten the operation of producing such explosive compound by dealing directly with the active ingredient in the first stage of manufacture, by which and by such means I retain the active properties and prevent the waste of the useful material. During the first stage of my process of manufacture desiccation of the material treated is unnecessary, and in the second stage such desiccation is minimized, and the time occupied in carrying out the process of manufacture is materially shortened.

By varying the proportion of the ingredients hereinafter described I manufacture a compound of greater or less explosive power, (according to the requirements of the material to be operated upon,) and the operation of mixing the ingredients can be performed by persons desirous of using the explosive, such operation being absolutely safe in the hands of inexperienced persons.

The manufacture of an explosive compound according to my process consists in the mix-

ture of picric acid with glycerine, and the combination of such compound with nitrate of potash, (or nitrate of sodium,) ground cedar or other suitable wood, and flowers of sulphur. In the first instance I dissolve picric acid in half its own weight of boiling glycerine, but may add additional quantities of picric acid if it is desired to produce greater solidity, and while in the state of solution I thoroughly mix it with twice its own weight of nitrate of potash, (or nitrate of sodium.) The mixture becomes solidified or of a pasty nature when cooled. Ground cedar or other suitable wood is then heated and mixed in the dry condition with the before-mentioned mixture in the proportion of one pound of ground wood to every ounce of the mixture. The ground wood, when thus impregnated with the pasty material, is further treated by admixture with a boiling solution of nitrate of potash in the approximate proportion of two and three-quarters pounds of nitrate of potash to every pound of ground wood. I then add flowers of sulphur in the proportion of five parts of sulphur to eleven parts of the impregnated ground wood. I can dispense with the flowers of sulphur by increasing the volume or quantity of the mixture of picric acid and glycerine.

For the purpose of producing a compound of greater explosive power absolutely free from danger, I mix the picric acid and glycerine with nitrate of potash in the proportion of one-fourth of the former to three-fourths of the latter, which, when carefully solidified, can be made impervious to water by known methods.

The above process secures absolute safety in the process of manufacture and produces an explosive compound of great power, safe for the purposes of storage and carriage, and particularly adapted for blasting operations. The compound is not susceptible to explosion by friction and the other ordinary methods of obtaining explosion in the open air, it being absolutely necessary, when using the compound, to exclude it from atmospheric influences in order to bring about explosion.

Having thus described the nature of my said invention and how the same is to be carried into effect, what I claim is—

1. That improvement in the art of manufacturing explosive compounds containing picric acid and nitrate of potash or its equivalent which consists in first mixing the picric acid with boiling-hot glycerine, as and for the purpose herein set forth.
2. That improvement in the art of manufacturing explosive compounds containing picric acid and nitrate of potash or its equivalent which consists in adding to a mixture of picric acid with boiling-hot glycerine, after the same has cooled, nitrate of potash or its equivalent at normal temperature, ground wood in a dry state, and nitrate of potash at boiling temperature, as herein set forth.
3. A process of manufacturing explosive compounds containing picric acid and nitrate

of potash or its equivalent, which consists, first, in mixing the picric acid with boiling-hot glycerine; second, mixing with the acid and glycerine nitrate of potash or the equivalent and allowing the mixture to cool; third, mixing with the cooled mass ground wood, as cedar-wood, in a dry state; fourth, adding to the mixture boiling-hot nitrate of potash, and, fifth, adding to the mixture flowers of sulphur, substantially as herein set forth.

Dated this 21st day of June, 1889.

W. EVELYN LIARDÉT.

Witnesses:

JOHN J. STONE,  
*Civil Engineer, Sydney.*  
ARTHUR J. STONE.  
*Cadet Engineer, Sydney.*